# EUROPEAN PATENT SPECIFICATION

(11) **EP 0 225 051 B1**
(45) Date of publication and mention of the grant of the patent: **19.02.1992**
(21) Application number: 86308419.0
(22) Date of filing: 29.10.1986
(51) Int. Cl.: C23F 11/167, C23F 11/18, C02F 5/14, C23G 5/00

(54) **The treatment of aqueous systems**
Behandlung von wässrigen Systemen
Traitement de systèmes aqueux

(30) Priority: 29.10.1985 GB 8526590; 30.09.1986 GB 8623464
(43) Date of publication of application: 10.06.1987
(73) Proprietor: W.R. Grace & Co.-Conn., New York, New York 10036 (US)
(72) Inventor: Greaves, Brian, Runcorn Cheshire WA7 4AL (GB)
(74) Representative: Ellis-Jones, Patrick George Armine

(56) References cited:
- EP-A- 0 006 065
- AT-B- 332 699
- DE-A- 2 338 352
- DE-A- 2 635 295
- DE-A- 3 314 008
- US-A- 3 669 901
- US-A- 3 794 603
- US-A- 4 018 701

## Description

The present invention relates to the treatment of aqueous systems and, more particularly, to reducing or eliminating corrosion in aqueous systems.

Many different types of material have been employed to prevent or inhibit corrosion in aqueous systems. These include inorganic salts such as nitrites and chromates, inorganic mono and polyphosphates, certain water soluble polymers including naturally occurring materials such as lignins and starches as well as synthetic materials such as polyacrylates, as well as organic phosphonates. In addition, it is well known to use zinc salts for this purpose. Indeed, it is known to use zinc salts in combination with organic type corrosion inhibitors, principally organic phosphonates and polyacrylates.

The use of zinc salts enables one to passivate corrosion of the metal in contact with the system. It is generally believed that localised high concentrations of hydroxide ions arise at sites of corrosion on the metal surface because, due to the galvanic cell effect, oxygen present in the water is reduced to hydroxide ions at the cathodic sites. These hydroxide ions then react with zinc ions of the zinc salt to give zinc hydroxide which in turn yields a protective film on the metal surface.

While this passivation system works reasonably satisfactorily in some aqueous media it is known that the use of zinc salts, with or without the organic type corrosion inhibitor, is ineffective when the pH of the system is high, for example at pH from 8.2 to 9.0. Such a pH can be present when the water is hard, or is otherwise alkaline ie of low hardness and high alkalinity as can be the case with base exchanged water. Under such circumstances, the zinc hydroxide precipitates prematurely in the system water and therefore does not form a protective film over the metal. Thus in such systems the zinc actually becomes a foulant of the system. Similar problems arise when the temperature of the aqueous system is raised, for example to at least 40°C as can occur when the aqueous system is used as cooling water which comes into contact with hot metal surfaces. AT-B-332 699 discloses preventing corrosion using a phosphonate and, optionally, a zinc salt.

It has now surprisingly been found, according to the present invention, that more effective corrosion inhibition can be obtained when a zinc salt is used together with a class of phosphonate or similar material and, in addition, a specific class of chelant. It has been found that this combination is capable of being effective under a combination of severe pH and temperature conditions. It is considerably more effective than existing zinc/organic products on pre-corroded mild steel surfaces since the combination is capable of stifling existing corrosion as well as enabling much faster passivation of the rusty surface to be brought about. Thus the combination, as well as inhibiting corrosion, also acts as an on line cleaning agent by removing old rust.

According to the present invention there is provided a method of treating an aqueous system which comprises adding thereto a zinc salt, a chelant having the formula set out below and either a product containing at least one phosphorus-containing acid group and at least one carboxylic acid group or an acrylic, vinyl or allyl carboxylic acid polymer.

Generally, any water soluble zinc salt can be used in the present invention. Typical salts which can be used include zinc sulphate, zinc chloride, zinc nitrate and zinc acetate, zinc sulphate monohydrate and zinc chloride being particularly preferred.

The third component used in the present invention will, in general, be a phosphonate. Preferably, the materials used contain at least two acid groups, one of which is a phosphonate group and the other is a carboxylic acid group, at least the two said acid groups being attached to carbon atoms.

Preferred phosphonates include hydroxy phosphonoacetic acid and 2-phosphono butane-1,2,4-tricarboxylic acid, the latter being particularly preferred. Thus these preferred phosphonates possess the general formula
wherein R is hydrogen, alkyl, alkenyl or alkynyl having up to 4 carbon atoms; phenyl; cycloalkyl having 3 to 6 carbon atoms; benzyl; phenethyl or
wherein R' is hydrogen, alkyl having 1 to 4 carbon atoms or carboxyl, R" is hydrogen or methyl and R''' is carboxyl or phosphonate.

It is also possible to employ as the third component in the method a polymeric material and, in particular, carboxylic acid polymers which contain a chain phosphorus atom which forms part of an acid group. Thus these polymeric materials are preferably phosphino polycarboxylic acids, typically those having the formula
where N + M = 4 to 20
The molecular weight of such polymers is relatively low, generally below 5,000, the preferred molecular weight being from 250 to 750, especially about 500. A particularly suitable polymer is that sold as "Belclene 500", a registered Trade Mark of Ciba-Geigy.

It has also been found that a synergistic effect, although most pronounced when the phosphorus containing materials are used, can also be obtained when a polycarboxylic acid is used, typically one having a molecular weight from 1,000 to 5,000. Such polymers may be derived from acrylic, vinyl or allyl carboxylic monomers, typically acrylic, methacrylic, maleic, fumaric, itaconic, crotonic or cinnamic acid alone or with a suitable comonomer. Such comonomers include acrylamide, (meth)acrylate esters or hydroxy esters e.g. hydroxypropyl esters, vinyl pyrrolidone, vinyl acetate, acrylonitrile, vinyl methyl ether, 2-acrylamido-2-methyl-propane sulphonic acid, vinyl or allyl sulphonic acid and styrene sulphonic acid as well as cationic monomers such as diallyl dimethyl ammonium chloride, dimethylamino ethylacrylate or methacrylate, optionally quaternised with, for example, dimethyl sulphate or methyl chloride.
The chelants which can be used in the method of the present invention possess the formula
where R¹ is hydrogen, hydroxyethyl or carboxymethyl, preferably carboxymethyl, R² is hydrogen, hydroxyphenyl, preferably ortho-hydroxyphenyl, which is optionally methyl or sulphonic acid substituted, or carboxyl, R⁴ is hydrogen or carboxyl,
where R¹, R² and R⁴ are as defined above and
X is -(CH₂)₂- or - (CH₂)₃ - with the proviso that at least one of R² and R³ contains a hydroxyphenyl group. The phenyl groups may be substituted, if desired, preferably by one or more halogen atoms.

If the chelant is to be used in aqueous systems which possess a high pH and a relatively high temperature it is preferred that at least one of R¹, R² and R³ contains a hydroxyl group. Thus the most preferred chelants possess a nitrogen ligand, a carboxylic acid group and a hydroxyl group.

Preferred chelants for use in the present invention include N,N'-di(-2-hydroxybenzyl-)trimethylenediamine-N, N'-diacetic acid, N,N'ethylene-bis-[2-(2-hydroxy-4-methyl-phenyl)-glycine], ethylenediamine N, N'-bis-[2-hydroxyphenylacetic acid] and N, N-di(2-hydroxy-5-sulphonic acid benzyl)glycine which is especially preferred not only on account of its effectiveness but also on account of its excellent solubility properties which facilitate the formulation of compositions.

In general, from 1 to 10 parts by weight of chelant and from 4 to 6 parts by weight of the phosphorus containing compound are employed to 1 part of the zinc salt. While in certain circumstances it may be desirable to add the individual components separately, in other situations it will be convenient to add the components together in the form of a composition. Accordingly, the present invention also provides a composition suitable for addition to an aqueous system which comprises a water soluble zinc salt, a product containing at least one phosphorus containing acid group and at least one carboxylic acid group or an acrylic, vinyl or allyl carboxylic acid polymer, and a chelant. In such a situation, it may be desirable to add further quantities of chelant as required. Typically, the composition will be an aqueous formulation containing, generally, 1% to 2% by weight of zinc salt (as zinc), 4% to 10% by weight of the phosphorus containing material or polymer and 1% to 25% by weight, especially about 5% by weight, of the chelant.

A further surprising feature of the present invention is that the presence of the combination of chelant and phosphorus containing compound and/or acrylic vinyl or allyl carboxylic acid polymer enables one to reduce the amount of zinc salt. It is usual in the art to employ amounts of the order of 2 to 5ppm zinc. However, with ever increasing restrictions on concentrations of zinc in discharges there is a constant demand to reduce the amounts of zinc used. It has been found that by using the additional ingredients it is possible to reduce the amount of zinc to, say, about 1ppm for comparable effectiveness. In such circumstances it is preferred to employ about 4ppm of the phosphorus compound and about 2.5 to 5ppm of chelant. If, on the other hand, one uses 2.5ppm of zinc then it is preferred to use about 10ppm of phosphorus compound and about 5ppm of chelant.

It is also possible to use the combination of the present invention together with other ingredients including phosphates, biocides, yellow metal corrosion inhibitors such as benzotriazole and tolyltriazole as well as other polymers which act as dispersants such as polyacrylic acid, polymaleic acid and copolymers of maleic acid with styrene sulphonic acid. In particular, it has been found that the use of certain dispersants, especially a copolymer of methacrylic acid and acrylamide is particularly advantageous, especially one in which the mole ratio is about 1:3, and further enhances the corrosion protection given by the three component system. In general the molecular weight of the homopolymers will be 1,000 to 10,000 while that of the copolymers will be 1,000 to 50,000.

The use of a phosphate is particularly noteworthy since zinc phosphate is effective in low water hardness systems because the zinc phosphate itself gives protection. By using the chelant and phosphorus containing compound as well it is possible, as previously discussed, to use significantly lower quantities of zinc.

The following Examples further illustrate the present invention.

### Examples 1 to 34

In these Examples tests were carried out on a laboratory scale recirculating rig consisting of a plastic vessel holding 8 litres of water and connected by tubing to a circulating pump the water passing from the pump through a glass rack holding the metal test coupons ('line') and returning to the plastic vessel. Any evaporation was made up by the addition of de-ionised water. Metal test coupons were also suspended in the plastic vessel ('Pond'). The corrosion rate was calculated from the weight of metal lost during test. The water temperature was maintained by means of a heater/thermostat arrangement. The conditions of the test were as follows:
- System Water: : 150ppm Ca hardness/150ppm 'M' Alkalinity
- Water pH: : 8.8
- Water Temperature: : 54°C or 40°C (as stated)
- Flow Rate: Line: : 2 ft/sec
- Pond: : 0.2 ft/sec
- Duration of Test: : 3 days
- Initial Passivation: : 1 day at 3 times normal maintenance dose.

Examples No. 1 - 14 were carried out at 40°C.

### Examples 1 - 14 illustrate:

i) The blend of zinc/chelant/phosphonate is superior to zinc/phosphonate or zinc/chelant.
ii) the best chelants are Chelants 1, 2,3 and 9.
iii) Phosphonate 1 gives significantly better results than comparative Phosphonate 2.

### Examples 15 - 34 were carried out at 54°C.

Chelant 1 = N, N'-di(-2 hydroxybenzyl trimethylenediamine-N,N'-diacetic acid
Chelant 2 = N,N' Ethylene-bis- [2(2-hydroxy-4 methyl-phenyl) - glycine]
Chelant 3 = Ethylenediamine N, N'bis-[2 hydroxyl phenyl acetic acid]
Chelant 4 = Ethylenediamine tetraacetic acid.
Chelant 5 = N,N-di (2 hydroxy ethyl) glycine.
Chelant 6 = N-Hydroxyethyl,N,N' Ethylenediamine triacetic acid.
Chelant 7 = 2-hydroxyethyl iminodiacetic acid.
Chelant 8 = Diethylene triamine penta acetic acid.
Chelant 9 = N,N-di(2 hydroxy -5-sulphonic acid benzyl) glycine
Phosphonate 1 = 2-Phosphonobutane 1,2,4 tricarboxylic acid.
Phosphonate 2 = Hydroxy ethylidene di-phosphonic acid.
Phosphonate 3 = Hydroxy phosphonoacetic acid.
Phosphino 1 = Phosphino polyacrylic acid, M.Wt. approx 500 (sold commercially as "Belclene 500" Ciba Geigy).

- Polymer 1 =: Copolymer of methacrylic acid/acrylamide, mole ratio 1:3, M.Wt. 35,000.
- Polymer 2 =: Polyacrylic acid, M.Wt.1000.
- Polymer 3 =: Polyacrylic acid, M.Wt.4500.

### Examples 15 - 34 indicate:

i) The excellent corrosion inhibiting properties of the zinc/chelant/phosphonate combinations are maintained at the higher test temperature; this should be compared with Chelant 8 which does not contain a hydroxy group (Example 32). The excellent corrosion inhibition is also maintained when the phosphonate is replaced by the phosphino-polycarboxylic acid in the 3 component combination.
ii) The presence of Polymer 1, (Example 20), enhances the corrosion protection conferred by the 4 component blend over that given by the corresponding 3 component blend, (Example 19), without polymer.
iii) The improvement brought about by the presence of the chelant with the zinc/polyacrylic acid combination.

### Examples 35 to 43

These Examples illustrate the effect of longer term tests. These were carried out on a laboratory scale simulated open, evaporative, recirculating cooling water system incorporating mild steel heat exchanger together with feed and bleed facilities which enable the system to run at a given concentration factor throughout the 14 day test. The test conditions were as follows:
- System Water: : 160ppm Calcium hardness 50ppm Magnesium hardness 200ppm 'M' Alkalinity
- Water Temperature (Pond): : 50°C
- pH: : 8.8
- Flow Rate through heat exchanger: : 0.3 ft/sec
- Flow Rate through coupon chamber: : 1.5 ft/sec
- Heat flux on exchanger: : 75 kj/m⁻²/sec⁻¹
- Duration of test: : 14 days
- Initial passivation: : 3 x normal maintenance dose, allowed to decay from start of test.

It was noticed that when Chelant 2 was in use (Examples 35 to 38), the corrosion which initiated on the heat exchanger was rapidly stifled whereas in Example 40 corrosion spread throughout the test. Chelant 4 was largely ineffective; in fact, the results indicate aggression. This shows that this chelant is unsuitable where there is a heat exchanger giving a high surface temperature.

Example 42 in relation to Example 43 shows the effect of using Chelant 2 in enabling one to reduce the concentration of zinc/phosphate.

## Claims

1. A method of treating an aqueous system which comprises adding thereto a water-soluble zinc salt, a chelant which possesses the formula where R¹ is hydrogen, hydroxyethyl or carboxymethyl, R² is hydrogen, hydroxyphenyl, which is optionally methyl or sulphonic acid substituted, or carboxyl, R⁴ is hydrogen or carboxyl, where R¹, R² and R⁴ are as defined above and X is -(CH₂)₂₋ or -(CH₂)₃-; the phenyl groups being optionally further substituted by one or more halogen atoms, with the proviso that at least one of R² and R³ contains a hydroxyphenyl group, and either a product containing at least one phosphorus-containing acid group and at least one carboxylic acid group or an acrylic, vinyl or allyl carboxylic acid polymer.

2. A method according to claim 1 in which the zinc salt is zinc sulphate, zinc chloride, zinc nitrate or zinc acetate.

3. A method according to claim 1 or 2 in which the phosphonate has the general formula wherein R is hydrogen, alkyl, alkenyl or alkynyl having up to 4 carbon atoms; phenyl; cycloalkyl having 3 to 6 carbon atoms; benzyl; phenethyl or wherein R' is hydrogen, alkyl having 1 to 4 carbon atoms or carboxyl, R" is hydrogen or methyl and R''' is carboxyl or phosphonate.

4. A method according to claim 3 in which the phosphonate is hydroxy-phosphonoacetic acid or 2-phosphonobutane-1,2,4-tricarboxylic acid.

5. A method according to claim 1 or 2 in which the product containing at least one phosphorus-containing acid group and at least one carboxylic acid group is a phosphino polycarboxylic acid having the formula where N + M = 4 to 20.

6. A method according to claim 1 or 2 in which the polymer is a copolymer of acrylic, methacrylic, maleic, fumaric, itaconic, crotonic or cinnamic acid with acrylamide, an acrylate or methacrylate ester or hydroxy ester, vinyl pyrrolidone, vinyl acetate, acrylonitrile, vinyl methyl ether, 2-acrylamido-2-methyl-propane sulphonic acid, vinyl, allyl or styrene sulphonic acid, or diallyldimethyl ammonium chloride or dimethylamino ethyl acrylate or methacrylate, optionally quaternised with dimethyl sulphate or methyl chloride.

7. A method according to claim 1 or 2 in which the polymer is a polymer of acrylic acid, methacrylic acid, maleic acid, fumaric acid, itaconic acid or crotonic acid, having a molecular weight from 1000 to 5000.

8. A method according to any one of claims 1 to 7 in which R¹ is hydrogen or carboxymethyl, R² is hydroxyphenyl which is optionally methyl or sulphonic acid substituted, R³ is or -CH₂C₆H₃ (OH) (SO₃H), the phenyl groups being optionally further substituted by one or more halogen atoms.

9. A method according to any one of claims 1 to 7 in which the chelant is N,N'-di(2-hydroxybenzyl)-trimethylenediamine-N,N'-diacetic acid, N,N'ethyenebis-[2(2-hydroxy-4-methyl-phenyl)-glycine}, ethylenediamine N,N'-bis-[2-hydroxyphenylacetic acid] or N,N-di (2-hydroxy-5-sulphonic acid benzyl) glycine.

10. A method according to any one of the preceding claims in which the zinc salt is added in an amount to provide up to 5 ppm zinc.

11. A method according to claim 10 in which the zinc salt is added to provide up to 2 ppm zinc.

12. A method according to any one of the preceding claims in which 1 to 10 parts by weight of chelant are added per part by weight of the zinc salt.

13. A method according to any one of the preceding claims in which 4 to 6 parts by weight of the phosphorus and carboxylic acid group containing compound are added per part by weight of the zinc salt.

14. A method according to any one of the preceding claims in which the system water attains a temperature of at least 40° C.

15. A method according to any one of the preceding claims in which the system water attains a pH of at least 8.2.

16. A composition suitable for addition to an aqueous system which comprises a water-soluble zinc salt, a product containing at least one phosphorus-containing acid group and at least one carboxylic acid group or an acrylic, vinyl or allyl carboxylic acid polymer, and a chelant which possesses the formula where R¹ is hydrogen, hydroxyethyl or carboxymethyl, R² is hydrogen, hydroxyphenyl, which is optionally methyl or sulphonic acid substituted, or carboxyl, R⁴ is hydrogen or carboxyl, where R¹, R² and R⁴ are as defined above and X is -(CH₂)₂- or -(CH₂)₃-; the phenyl groups being optionally further substituted by one or more halogen atoms, with the proviso that at least one of R² and R³ contains a hydroxyphenyl group.

17. A composition according to claim 16 in which the zinc salt is zinc sulphate, zinc chloride, zinc nitrate or zinc acetate.

18. A composition according to claim 16 or 17 which is agueous and contains 1 to 2% by weight of zinc salt (as zinc), 4 to 10% by weight of the phosphorus and carboxylic acid group containing material or polymer and 1 to 25% by weight of the chelant.

19. A composition according to any one of claims 16 to 18 which also comprises a phosphate, biocide, yellow metal corrosion inhibitor or dispersant.

20. A composition according to claim 19 in which the dispersant is a copolymer of methacrylic acid and acrylamide.

21. A composition according to any one of claims 16 to 20 in which the phosphonate has the general formula wherein R is hydrogen, alkyl, alkenyl or alkynyl having up to 4 carbon atoms; phenyl; cycloalkyl having 3 to 6 carbon atoms; benzyl; phenethyl or wherein R' is hydrogen, alkyl having 1 to 4 carbon atoms or carboxyl, R'' is hydrogen or methyl and R''' is carboxyl or phosphonate.

22. A composition according to claim 21 in which the phosphonate is hydroxy-phosphonoacetic acid or 2-phosphonobutane-1,2,4-tricarboxylic acid.

23. A composition according to any one of claims 16 and 18 to 20 in which the product containing at least one phosphorus-containing acid group and at least one carboxylic acid group is a phosphino polycarboxylic acid having the formula where N + M = 4 to 20.

24. A composition according to any one of claims 16 and 18 to 20 in which the polymer is a copolymer of acrylic, methacrylic, maleic, fumaric, itaconic, crotonic or cinnamic acid with acrylamide, an acrylate or methacrylate ester or hydroxy ester, vinyl pyrrolidine, vinyl acetate, acrylonitrile, vinyl methyl ether, 2-acrylamido--2-methyl-propane sulphonic acid, vinyl, allyl or styrene sulphonic acid, or diallyldimethyl ammonium chloride or dimethylamino ethyl acrylate or methacrylate, optionally quaternised with dimethyl sulphate or methyl chloride.

25. A composition according to any one of claims 16 and 18 to 20 in which the polymer is a polymer of acrylic acid, methacrylic acid, maleic acid, fumaric acid, itaconic acid or crotonic acid, having a molecular weight from 1000 to 5000.

26. A composition according to any one of claims 16 to 25 in which R¹ is hydrogen or carboxymethyl, R² is hydroxyphenyl which is optionally methyl or sulphonic acid substituted, R³ is or -CH₂C₆H₃ (OH)(SO₃H), the phenyl groups being optionally further substituted by one or more halogen atoms.

27. A composition according to any one of claims 16 to 26 in which the chelant is N,N'-di(2-hydroxybenzyl)-trimethyl-enediamine-N,N'-diacetic acid, N,N'ethylenebis-[2(2-hydroxy-4-methyl-phenyl)-glycine], ethylenediamine N,N'-bis-[2-hydroxyphenylacetic acid] or N,N-di(2-hydroxy-5-sulphonic acid benzyl) glycine.

## Revendications

1. Procédé de traitement d'un système aqueux qui consiste à ajouter à ce système un sel de zinc soluble dans l'eau, un chélateur qui possède la formule où R¹ est hydrogène, hydroxyéthyle ou carboxyméthyle, R² est hydrogène, hydroxyphényle, qui est facultativement substitué par méthyle ou l'acide sulfonique, ou carboxyle, R⁴ est hydrogène ou carboxyle, R³ est où R¹ , R² et R⁴ sont comme définis ci-dessus et X est -(CH₂)₂- ou -(CH₂)₃- ; les groupes phényle étant facultativement encore substitués par un ou plusieurs atomes d'halogène, à la condition qu'au moins l'un des R² et R³ contienne un groupe hydroxyphényle, et soit un produit contenant au moins un groupe acide contenant du phosphore et au moins un groupe acide carboxylique ou un polymère d'acide carboxylique acrylique, vinylique ou allylique.

2. Procédé suivant la revendication 1, dans lequel le sel de zinc est le sulfate de zinc, le chlorure de zinc, le nitrate de zinc ou l'acétate de zinc.

3. Procédé suivant la revendication 1 ou 2, dans lequel le phosphonate a la formule générale : où R est hydrogène, alkyle, alcényle ou alkynyle ayant jusqu'à 4 atomes de carbone ; phényle ; cycloalkyle ayant de 3 à 6 atomes de carbone ; benzyle ; phénéthyle ou dans laquelle R' est hydrogène, alkyle ayant de 1 à 4 atomes de carbone ou carboxyle, R" est l'hydrogène ou méthyle et R''' est carboxyle ou phosphonate.

4. Procédé suivant la revendication 3, dans lequel le phosphonate est l'acide hydroxy-phosphonoacétique ou l'acide 2-phosphonobutane-1,2,4-tricarboxylique.

5. Procédé suivant la revendication 1 ou 2, dans lequel le produit contenant au moins un groupe acide contenant du phosphore et au moins un groupe acide carboxylique est un acide phosphino-polycarboxylique ayant la formule où N + M = 4 à 20.

6. Procédé suivant la revendication 1 ou 2, dans lequel le polymère est un copolymère d'acide acrylique, méthacrylique, maléïque, fumarique, itaconique, crotonique ou cinnamique avec l'acrylamide, un ester d'acrylate ou de méthacrylate ou un ester hydroxy, la vinyl-pyrrolidone, l'acétate de vinyle, l'acrylonitrile, le vinyl méthyléther, l'acide 2-acrylamido-2-méthyl-propane sulfonique, l'acide sulfonique de vinyle, allyle ou styrène, ou le chlorure de diallyldiméthyl ammonium ou le méthacrylate ou acrylate de diméthylamino éthyle, facultativement quaternisés avec du sulfate de diméthyle ou du chlorure de méthyle.

7. Procédé suivant la revendication 1 ou 2, dans lequel le polymère est un polymère d'acide acrylique, d'acide méthacrylique, d'acide maléïque, d'acide fumarique, d'acide itaconique ou d'acide crotonique, ayant un poids moléculaire entre 1.000 et 5.000.

8. Procédé suivant l'une quelconque des revendications 1 à 7, dans lequel R¹ est hydrogène ou carboxyméthyle, R² est hydroxyphényle qui est facultativement substitué par méthyle ou l'acide sulfonique, R³ est ou -CH₂C₆H₃(OH)(SO₃H), les groupes phényle étant en outre facultativement substitués par un ou plusieurs atomes d'halogène.

9. Procédé suivant l'une quelconque des revendications 1 à 7, dans lequel le chélateur est l'acide N,N'-di(2-hydroxybenzyl)-triméthylènediamine-N,N'-diacétique, la N,N'éthylènebis-[2(2-hydroxy-4-méthylphényl)-glycine], l'éthylènediamine N,N'-bis[2-acide hydroxyphénylacétique] ou la N,N-di(2-hydroxy-5-benzyle acide sulfonique)glycine.

10. Procedé suivant l'une des revendications précédentes, dans lequel le sel de zinc est ajouté suivant une quantité procurant jusqu'à 5 ppm de zinc.

11. Procédé suivant la revendication 10, dans lequel le sel de zinc est ajouté pour procurer jusqu'à 2 ppm de zinc.

12. Procédé suivant l'une des revendications précédentes, dans lequel de 1 à 10 parties en poids de chélateur sont ajoutées par partie en poids du sel de zinc.

13. Procédé suivant l'une des revendications précédentes, dans lequel de 4 à 6 parties en poids du composé contenant un groupe acide carboxylique et du phosphore sont ajoutées par partie en poids du sel de zinc.

14. Procédé suivant l'une des revendications précédentes, dans lequel l'eau du système atteint une température d'au moins 40°C.

15. Procédé suivant l'une des revendications précédentes, dans lequel l'eau du système atteint un pH d'au moins 8,2.

16. Composition appropriée pour addition à un système aqueux, qui comprend un sel de zinc soluble dans l'eau, un produit contenant au moins un groupe acide contenant du phosphore et au moins un groupe acide carboxylique ou un polymère d'acide carboxylique acrylique, vinylique ou allylique, et un chélateur qui possède la formule où R¹ est hydrogène, hydroxyéthyle ou carboxyméthyle, R² est hydrogène, hydroxyphényle, qui est facultativement substitué par méthyle ou l'acide sulfonique, ou carboxyle, R⁴ est hydrogène ou carboxyle, R³ est où R¹ , R² et R⁴ sont comme définis ci-dessus et X est-(CH₂)₂ - ou -(CH₂)₃- ; les groupes phényle étant en outre facultativement substitués par un ou plusieurs atomes d'halogène, à la condition qu'au moins l'un des R² et R³ contienne un groupe hydroxyphényle.

17. Composition suivant la revendication 16, dans laquelle le sel de zinc est le sulfate de zinc, le chlorure de zinc, le nitrate de zinc ou l'acétate de zinc.

18. Composition suivant la revendication 16 ou 17, qui est aqueuse et contient 1 à 2% en poids de sel de zinc (comme zinc) de 4 à 10% en poids du polymère ou matériau contenant le groupe acide carboxylique et le phosphore et de 1 à 25% en poids du chélateur.

19. Composition suivant l'une des revendications 16 à 18, qui comprend également un phosphate, un biocide, un dispersant ou un inhibiteur jaune de corrosion du métal.

20. Composition suivant la revendication 19, dans laquelle le dispersant est un copolymère d'acide méthacrylique et d'acrylamide.

21. Composition suivant l'une des revendications 16 à 20, dans laquelle le phosphonate a la formule générale où R est hydrogène, alkyle, alcényle ou alkynyle ayant jusqu'à 4 atomes de carbone ; phényle ; cycloalkyle ayant de 3 à 6 atomes de carbone ; benzyle ; phénéthyle ou où R' est hydrogène, alkyle ayant de 1 à 4 atomes de carbone ou carboxyle, R" est hydrogène ou méthyle et R''' est carboxyle ou phosphonate.

22. Composition suivant la revendication 21, dans laquelle le phosphonate est l'acide hydroxyphosphonoacétique ou l'acide 2-phosphonobutane-1,2,4-tricarboxylique.

23. Composition suivant l'une quelconque des revendications 16 et 18 à 20, dans laquelle le produit contenant au moins un groupe acide contenant du phosphore et au moins un groupe acide carboxylique est un acide phosphino-carboxylique possédant la formule où N + M = 4 à 20.

24. Composition suivant l'une des revendications 16 et 18 à 20, dans laquelle le polymère est un copolymère d'acide acrylique, méthacrylique, maléïque, fumarique, itaconique, crotonique ou cinnamique avec de l'acrylamide, un ester de méthacrylate ou d'acrylate ou un ester hydroxy, la vinyl-pyrrolidine, l'acétate de vinyle, l'acrylonitrile, le vinyl méthyléther, l'acide 2-acrylamido-2-méthyl-propane sulfonique, l'acide sulfonique de vinyle, allyle ou styrène, ou le chlorure de diallyldiméthyl ammonium ou le méthacrylate ou acrylate de diméthylamino éthyle, facultativement quaternisés avec du sulfate de diméthyle ou du chlorure de méthyle.

25. Composition suivant l'une des revendications 16 et 18 à 20, dans laquelle le polymère est un polymère d'acide acrylique, d'acide méthacrylique, d'acide maléïque, d'acide fumarique, d'acide itaconique ou d'acide crotonique, ayant un poids moléculaire compris entre 1.000 et 5.000.

26. Composition suivant l'une quelconque des revendications 16 à 25, dans laquelle R¹ est hydrogène ou carboxyméthyle, R² est hydroxyphényle qui est facultativement substitué par méthyle ou l'acide sulfonique, R³ est ou -CH₂C₆H₃(OH)(SO₃H), les groupes phényle étant en outre facultativement substitués par un ou plusieurs atomes d'halogène.

27. Composition suivant l'une quelconque des revendications 16 à 26, dans laquelle le chélateur est l'acide N,N'-di(2-hydroxybenzyl)-triméthylènediamine-N,N'-diacétique, la N,N'-éthylènebis[2(2-hydroxy-4-méthylphényl)-glycine], l'éthylènediamine N,N'-bis-[2-acide hydroxyphénylacétique] ou la N,N-di(2-hydroxy-5-acide sulfonique benzyle)glycine.

## Patentansprüche

1. Verfahren zur Behandlung eines wäßrigen Systems, bei dem diesem System ein wasserlösliches Zinksalz, ein Chelatbildner mit der Formel wobei R¹ Wasserstoff, Hydroxyethyl oder Carboxymethyl ist, R² Wasserstoff, Hydroxyphenyl, das gegebenenfalls methyl- oder sulfonsäuresubstituiert ist, oder Carboxyl ist, R⁴ Wasserstoff oder Carboxyl ist, ist, wobei R¹, R² und R⁴ wie oben definiert sind und X -(CH₂)₂- oder -(CH₂)₃- ist, die Phenylgruppen gegebenenfalls außerdem durch ein oder mehrere Halogenatome substituiert sind, mit der Maßgabe, daß mindestens R² oder R³ eine Hydroxyphenylgruppe enthält, und entweder ein Produkt, das mindestens eine Phosphor enthaltende Säuregruppe und mindestens eine Carbonsäuregruppe enthält, oder ein Acryl-, Vinyl- oder Allylcarbonsäurepolymer zugesetzt wird.

2. Verfahren nach Anspruch 1, bei dem das Zinksalz Zinksulfat, Zinkchlorid, Zinknitrat oder Zinkacetat ist.

3. Verfahren nach Anspruch 1 oder 2, bei dem das Phosphonat die allgemeine Formel hat, wobei R Wasserstoff, Alkyl, Alkenyl oder Alkinyl mit bis zu 4 Kohlenstoffatomen, Phenyl, Cycloalkyl mit 3 bis 6 Kohlenstoffatomen, Benzyl Phenetyl oder ist, wobei R' Wasserstoff, Alkyl mit 1 bis 4 Kohlenstoffatomen oder Carboxyl ist, R" Wasserstoff oder Methyl ist und R'" Carboxyl oder Phosphonat ist.

4. Verfahren nach Anspruch 3, bei dem das Phosphonat Hydroxyphosphonessigsäure oder 2-Phosphonbutan-1,2,4-tricarbonsäure ist.

5. Verfahren nach Anspruch 1 oder 2, bei dem das mindestens eine Phosphor enthaltende Säuregruppe und mindestens eine Carbonsäuregruppe enthaltende Produkt, eine Phosphinpolycarbonsäure mit der Formel mit N + H = 4 bis 20 ist.

6. Verfahren nach Anspruch 1 oder 2, bei dem das Polymer ein Copolymer aus Acryl-, Methacryl-, Malein-, Fumar-, Itacon-, Croton- oder Zimtsäure mit Acrylamid, einem Acrylat- oder Methacrylatester oder Hydroxyester, Vinylpyrrolidon, Vinylacetat, Acrylnitril, Vinylmethylether, 2-Acrylamido--2methyl-propansulfonsäure, Vinyl-, Allyl- oder Styrolsulfonsäure, Diallyldimethylammoniumchlorid oder Dimethylaminoethylacrylat oder -methacrylat, gegebenenfalls quaternisiert mit Dimethylsulfat oder Methylchlorid, ist.

7. Verfahren nach Anspruch 1 oder 2, bei das Polymer ein Polymer aus Acrylsäure, Methacrylsäure, Maleinsäure, Fumarsäure, Itaconsäure oder Crotonsäure mit einem Molekulargewicht von 1 000 bis 5 000 ist.

8. Verfahren nach einem der Ansprüche 1 bis 7, bei dem R¹ Wasserstoff oder Carboxymethyl ist, R² Hyxdroxyphenyl ist, das gegebenenfalls methyl- oder sulfonsäuresubstituiert ist, oder -CH₂C₆H₃(OH)(SO₃H) ist, wobei die Phenylgruppen gegebenenfalls außerdem durch ein oder mehrere Halogenatome substituiert sind.

9. Verfahren nach einem der Ansprüche 1 bis 7, bei dem der Chelatbildner N, N'-Di(2-hydroxybenzyl)-trimethylendiamin-N,N'-diessigsäure, N,N'-Ethylen-bis[2(2-hydroxy-4-methylphenyl)glycin], Ethylendiamin - N, N'-bis [2-hydroxyphenylessigsäure] oder N,N-Di(2-hydroxy-5-sulfonsäurebenzyl)glycin ist.

10. Verfahren nach einem der vorhergehenden Ansprüche, bei dem das Zinksalz in einer solchen Menge zugesetzt wird, daß es bis zu 5 ppm Zink liefert.

11. Verfahren nach Anspruch 10, bei dem das Zinksalz zugesetzt wird, um bis zu 2 ppm Zink zu liefern.

12. Verfahren nach einem der vorhergehenden Ansprüche, bei dem 1 bis 10 Gewichtsteile Chelatbildner pro Gewichtsteil Zinksalz zugesetzt werden.

13. Verfahren nach einem der vorhergehenden Ansprüche, bei dem 4 bis 6 Gewichtsteile der Phosphor und Carbonsäuregruppe enthaltenden Verbindung pro Gewichtsteil Zinksalz zugesetzt werden.

14. Verfahren nach einem der vorhergehenden Ansprüche, bei dem das Systemwasser eine Temperatur von mindestens 40°C erreicht.

15. Verfahren nach einem der vorhergehenden Ansprüche, bei dem das Systemwasser einen pH-Wert von mindestens 8,2 erreicht.

16. Zum Zusetzen zu einem wäßrigen System geeignete Zusammensetzung, die ein wasserlösliches Zinksalz, ein Produkt mit mindestens einer Phosphor enthaltenden Säuregruppe und mindestens einer Carbonsäuregruppe oder ein Acryl-, Vinyl- oder Allylcarbonsäurepolymer und einen Chelatbildner mit der Formel umfaßt, wobei R¹ Wasserstoff, Hydroxyethyl oder Carboxymethyl ist, R² Wasserstoff, Hydroxyphenyl, das gegebenenfalls methyl- oder sulfonsäuresubstituiert ist, oder Carboxyl ist, R⁴ Wasserstoff oder Carboxyl ist, ist, wobei R¹, R² und R⁴ wie oben definiert sind und X -(CH₂)₂- oder -(CH₂)₃- ist, und die Phenylgruppen gegebenenfalls außerdem durch ein oder mehrere Halogenatome substituiert sind, mit der Maßgabe, daß mindestens R² oder R³ eine Hydroxyphenylgruppe enthält.

17. Zusammensetzung nach Anspruch 16, bei der das Zinksalz Zinksulfat, Zinkchlorid, Zinknitrat oder Zinkacetat ist.

18. Zusammensetzung nach Anspruch 16 oder 17, die wäßrig ist und 1 bis 2 Gew.-% Zinksalz (als Zink), 4 bis 10 Gew.-% Phosphor und Carbonsäuregruppe enthaltendes Material oder Polymer und 1 bis 25 Gew.-% Chelatbildner enthält.

19. Zusammensetzung nach einem der Ansprüche 16 bis 18, die außerdem ein Phosphat, Biozid, gelben Metallkorrosionsinhibitor oder Dispergiermittel umfaßt.

20. Zusammensetzung nach Anspruch 19, bei der das Dispergiermittel ein Copolymer aus Methacrylsäure und Acrylamid ist.

21. Zusammensetzung nach einem der Ansprüche 16 bis 20, bei der das Phosphonat die allgemeine Formel hat, wobei R Wasserstoff, Alkyl, Alkenyl oder Alkinyl mit bis zu 4 Kohlenstoffatomen, Phenyl, Cycloalkyl mit 3 bis 6 Kohlenstoffatomen, Benzyl, Phenetyl oder ist, wobei R' Wasserstoff, Alkyl mit 1 bis 4 Kohlenstoffatomen oder Carboxyl ist, R" Wasserstoff oder Methyl ist und R"' Carboxyl oder Phosphonat ist.

22. Zusammensetzung nach Anspruch 21, bei der das Phosphonat Hydroxyphosphonessigsäure oder 2-Phosphonbutan-1,2,4-tricarbonsäure ist.

23. Zusammensetzung nach einem der Ansprüche 16 und 18 bis 20, bei der das mindestens eine Phosphor enthaltende Säuregruppe und mindestens eine Carbonsäuregruppe enthaltende Produkt eine Phosphinpolycarbonsäure mit der Formel mit N + M = 4 bis 20 ist.

24. Zusammensetzung nach einem der Ansprüche 16 und 18 bis 20, bei der das Polymer ein Copolymer aus Acryl-, Methacryl-, Malein-, Fumar-, Itakon-, Croton- oder Zimtsäure mit Acrylamid oder einem Acrylat- oder Methacrylatester oder Hydroxyester, Vinylpyrrolidin, Vinylacetat, Acrylnitril, Vinylmethylether, 2-Arylamido-2-methyl-propansulfonsäure, Vinyl-, Allyl- oder Styrolsulfonsäure, Diallyldimethylammoniumchlorid oder Dimethylaminoethylacrylat oder -methacrylat, gegebenenfalls quaternisiert mit Dimethylsulfat oder Methylchlorid, ist.

25. Zusammensetzung nach einem der Ansprüche 16 und 18 bis 20, bei der das Polymer ein Polymer aus Acrylsäure, Methacrylsäure, Maleinsäure, Fumarsäure, Itakonsäure oder Crotonsäure mit einem Molekulargewicht von 1 000 bis 5 000 ist.

26. Zusammensetzung nach einem der Ansprüche 16 bis 25, bei der R¹ Wasserstoff oder Carboxymethyl ist, R² Hydroxyphenyl ist, das gegebenenfalls methyl- oder sulfonsäuresubstituiert ist, oder -CH₂C₆H₃(OH)(SO₃H) ist, wobei die Phenylgruppen gegebenenfalls außerdem durch ein oder mehrere Halogenatome substituiert sind.

27. Zusammensetzung nach einem der Ansprüche 16 bis 26, bei der der Chelatbildner H, N'-Di(2-hydroxybenzyl)-trimethylendiamin-N,N'-diessigsäure, N,N'-Ethylen - bis [2 (2-hydroxy-4-methyl-phenyl)glycin], Ethylendiamin - N,N'-bis [2-hydroxyphenylessigsäure] oder N,N'-Di(2-hydroxy-5-sulfonsäurebenzyl)glycin ist.
